

## UNITED STATES PATENT OFFICE

ADOLF BECK, OF BITTERFIELD, AND HUGO DIBELKA, OF DUSSELDORF-OBERKASSEL, GERMANY, ASSIGNEES, BY MESNE ASSIGNMENTS, TO MAGNESIUM DEVELOPMENT CORPORATION, A CORPORATION OF DELAWARE

PROCESS FOR THE TREATMENT OF ARTICLES MADE OF MAGNESIUM OR HIGH PERCENTAGE MAGNESIUM ALLOYS

No Drawing. Application filed July 20, 1932, Serial No. 379,871, and in Germany July 25, 1928.

This invention relates to a process for improving the resistance to corrosion of magnesium and magnesium alloys. It is well known that a large number of liquids including water exercise a corroding influence on magnesium and its alloys and it is an object of our present invention to lessen or even completely inhibit this corrosive action so as to enable articles made of said metals to be employed for various purposes from which they were hitherto precluded owing to their liability to corrode.

We have ascertained that in certain cases in which the surface of articles consisting mainly of magnesium comes into contact with a corroding liquid, such as water, only temporarily, during their employment, a special treatment as was hitherto generally applied with the object of forming a protective coating for preventing corrosion on the metal can be dispensed with. This also applies even if the water has not the same degree of purity as distilled water. We have discovered that it is merely necessary to add to the water coming into contact with the articles during their employment a small percentage, approximately 1%, of a soluble dichromate, preferably dichromate of potassium.

0 A particular instance of this kind is the treatment of sheets of magnesium alloys in the wetting appliance of offset printing machines, though we wish it to be understood that the applicability of our invention is, by 5 no means, limited to this purpose.

We claim:

1. The process for preventing the corrosive action of water on magnesium or magnesium alloys which comprises adding to the water a small amount, approximating 1%, of a water soluble dichromate.
2. The process as defined in claim 1 wherein the water soluble dichromate is potassium dichromate.
- 5 In testimony whereof we have hereunto set our hands.

ADOLF BECK.  
HUGO DIBELKA.